# EUROPEAN PATENT SPECIFICATION

(11) **EP 0 276 371 B1**
(45) Date of publication and mention of the grant of the patent: **20.03.1991**
(21) Application number: 87114670.0
(22) Date of filing: 08.10.1987
(51) Int. Cl.: C23C 22/04, C23C 22/03

(54) **Process for treating metal surface**
Verfahren zur Behandlung von Metalloberflächen
Procédé de traitement de surfaces métalliques

(30) Priority: 09.01.1987 JP 1824/87
(43) Date of publication of application: 03.08.1988
(73) Proprietor: Nippon Dacro Shamrock Co. Ltd., Yokohama, Kanagawa-ken (JP)
(72) Inventor: Nishikawa, Toshio, Yokohama Kanagawa-ken (JP); Ayukawa, Nobuhiro, Kamakura Kanagawa-ken (JP)
(74) Representative: Strehl Schübel-Hopf Groening & Partner

(56) References cited:
- EP-A- 0 089 456
- EP-A- 0 170 988
- FR-A- 2 304 684
- FR-A- 2 304 685
- US-A- 2 927 046
- US-A- 3 285 788
- US-A- 3 437 531

## Description

### Field of the Invention

This invention relates to a process for treating metal surface, by which corrosion resistance of the metal and adhesion of coating thereto are improved.

### Background of the Invention

It is known to phosphate a metal surface, and subject the thus formed phosphate film to chromic acid chemical conversion treatment (often called "chromium rinsing") in order to improve the corrosion resistance of the metal and adhesion of coating thereto.

In the early days, these two treatments were carried out using aqueous treating compositions. Such a process comprising phosphating and chromium rinsing requires a plurality of treating steps and a large space for the equipment, consumes a large amount of energy for evaporating water, and above all, is accompanied by problems of environmental pollution caused by aqueous waste. Therefore, recently, these treatments are mainly carried out using non-aqueous treating compositions. Such a typical process for this is disclosed in Japanese Patent Publication No. 42-3363 (1967). However, as the organic solvent for the compositions for the two treatments, only chlorinated hydrocarbon has been used.

The respective compositions per se have been improved, and there is known a phosphating treatment composition consisting of 100 parts by weight of a halogenated hydrocarbon solvent (carbon tetrachloride, chloroform, methylene chloride, 1,1,1-trichloroethane, trichloroethylene, perchloroethylene, trichlorotrifluoroethylene, perchloroethylene, trichlorotrifluoroethane, tetrachlorodifluoroethane, dichlorotetrafluoroethane, trifluoromonofluoromethane, etc. or a mixture thereof), 0.05-5 parts by weight of phosphoric acid compound such as orthophosphoric acid, pyrophosphoric acid, polyphosphoric acid such as triphosphoric acid, a salt thereof, an acidic metal salt of phosphoric acid, an acidic alkyl ester of phosphoric acid, or a mixture thereof), 1-75 parts by weight of an alcohol solubilizer having 1-10 carbon atoms such as methanol, ethanol, isopropyl alcohol, n-propanol, n-butanol, sec-butanol, t-butanol, etc. and 0.01-2 parts by weight of a nitrogen-containing organic compound reaction promoter, urea, pyridine, thiourea, dimethylisobutylenamine, ethylenediamine tetraacetate, dinitrotoluene, etc. This phosphating composition may contain a small amount of a quinone, an aromatic compound having a nitroso or azo functional group or a zinc compound such as zinc phosphate, zinc fluoride, zinc oxide, a fatty acid salt of zinc, etc. as a stabilizer for halogenated hydrocarbon solvent. The phosphating composition may further contain 0.5-15 parts by weight of aprotic polar organic compound such as N,N-dimethylformamide, dimethylsulfoxide, acetonitrile, acetone, nitromethane, nitrobenzene and tetramethylenesulfone. The phosphating composition may still further contain not less than 0.4 part by weight and not more than 5 parts by weight of water (in an amount that maintains a homogeneous phase). Water acts as a reaction promoter. (Japanese Patent Publication Nos. 57-49111, 56-31878, etc.)

Japanese Laying-Open Patent Publication No. 61-34184 of the applicant of the present application discloses a metal-surface-treating solution consisting of 100 parts by weight of a chlorofluorinated hydrocarbon organic solvent (typically, trichlorotrifluoroethane, tetrachlorodifluoroethane, tetrachlorodifluoroethane, dichlorotetrafluoroethane, trichloromonofluoromethane, etc. or a mixture thereof), 0.01-10 part by weight of chromic acid anhydride, 0.001-0.1 part by weight of an organic acid having 1-20 carbon atoms (typically, formic acid, acetic acid, lactic acid, stearic acid, oxalic acid, fumaric acid, naleic acid, malic acid, etc.) and 1-20 parts by weight of an alcohol solubilizer having 3-20 carbon atoms (typically isopropyl alcohol, tert-butanol, tert-amyl alcohol, triphenyl carbinol, etc. or a mixture thereof). In this case, an organic acid reaction promoter can be dispensed with.

Up to today, however, in the combination of the phosphating treatment and the chromic acid chemical conversion treatment, there has been no case wherein a chromic acid chemical conversion treatment composition using a fluorochlorinated hydrocarbon as a solvent is used.

We have found that in the combination of the phosphating treatment and the chromic acid chemical conversion treatment, if at least the chromic acid chemical conversion treatment is carried out using a chromic acid chemical conversion treatment solution in which a fluorochlorinated hydrocarbon is used as the solvent, the treated metal surface exhibits excellent adhesion property to coatings (paints).

### Disclosure of the Invention

This invention provides a process for treating metal surface comprising subjecting a metal surface to phosphating treatment and subjecting the phosphated surface to chromic acid chemical conversion treatment, said process being characterized in that the phosphating treatment is carried out using a non-aqueous phosphating treatment solution in which a chlorinated or chlorofluorinated hydrocarbon is used as the solvent and the chromic acid chemical conversion treatment is carried out using a non-aqueous chromic acid chemical conversion treatment solution in which a chlorofluorinated hydrocarbon is used as the solvent.

In the process of the present invention, the phosphating treatment composition per se is known as stated above.

In the process of the present invention, the chromic acid chemical conversion composition per se is also known as stated above.

The process of the present invention is applicable to all the metals to which the known phosphating treatment and chromic acid chemical conversion treatment are applicable, that is, iron and steel, zinc, aluminum, tin and alloys thereof.

### Specific Description of the Invention

Now the invention will be described in detail by way of working examples and comparative examples. It should be understood that the invention is not limited to these working examples only.

### Example 1

A phosphating treatment solution consisting of 100 parts by weight (hereinafter referred to simply as parts) trichlorotrifluoroethane, 22 parts methanol and 0.6 part orthophosphoric acid and 4 parts N,N-dimethylformamide was kept at the boiling temperature thereof. Test panels (70 x150 x 0.8 mm cold-rolled steel sheets) which had been degreased and cleansed beforehand were immersed in the boiling solution for 1 minute, were thereafter washed with the vapor in the vapor zone above the treating solution, and then were dried in the vapor-free space above the vapor zone. (Phosphating treatment)

Then, a chromic acid chemical conversion treatment solution consisting of 100 parts trichlorotrifluoroethane, 5 parts t-amyl alcohol, and 1 part chromic acid anhydride was kept at the boiling temperature thereof, and the test panels which had been phosphated as described above were immersed in the boiling treating solution for 15 seconds, and then were dried in the vapor-free space. (Chromic acid chemical conversion treatment)

The thus treated panels were coated with an epoxy resin powder paint ("Konac No. 3500" manufactured by Nippon Oil and Fats Company, Ltd.) or an acrylic resin powder paint ("Konac No. 4500" manufactured by Nippon Oil and Fats Company, Ltd.) by the electrostatic painting process, and the thus painted panels were baked at 180°C for 20 minutes.

The adhesion of the paint was tested by scoring some of the painted panels in a grid pattern at intervals of 1 mm reaching the substrate, forming 100 small squares by means of a knife edge, applying a cellophane adhesive tape 20 mm in width (manufactured by Nichiban Co.) onto the scored surface and peeling off the tape quickly at an angle of 45°. The number of the remaining squares of the coating (paint) was counted and the adhesion of the coating film before the corrosion test (named primary adhesion) was evaluated.

Other coated (painted) panels were scored in an X pattern (called cross cutting), and the panels were subjected to the salt spray test to investigate the corrosion resistance performance of the coating.

Occurrence of blisters at the cross-cutting was observed (the width of blisters formed along the cutting (score) was measured), and the adhesion of the coating film after the corrosion test (called "secondary adhesion") was measured by the cellophane adhesive tape test. (Width of the peeled-off zone of the coating was measured and the number of the remaining squares was counted.)

The results are indicated in Table 1 together with the results of Example 1a, Comparative Example 1 and Comparative Example 1a described hereinafter.

### Example 1a

Example 1 was repeated using the same chromic acid chemical conversion treatment composition which had been continuously used for 12 months.

### Comparative Example 1

The procedure of Example 1 was repeated using a conventional chromic acid chemical conversion treatment composition in which methylene chloride (chlorinated hydrocarbon) was used as the solvent instead of the composition in which the fluorochlorinated hydrocarbon solvent was used.

### Comparative Example 1a

The procedure of Example 1 was repeated using the same chromic acid chemical conversion treatment composition as used in Comparative Example 1 (using the chlorinated hydrocarbon) which had been continuously used for one week.

### Example 2

Test panels of the same kind as used in Example 1 were phosphated in the same manner as in Example 1. Then the thus phosphated panels were immersed in a fresh chromic acid chemical conversion treatment solution consisting of 100 parts trichlorotrifluoroethane, 5 parts t-amyl alcohol, and 0.05 part chromic acid anhydride, which was kept at the boiling temperature thereof, for 30 seconds, and then dried in the vapor-free space above the solution.

The thus treated panels were coated with the same epoxy and acrylic resin powder paints as used in Example 1 and the primary adhesion and the secondary adhesion were respectively measured.

The results are indicated in Table 2 together with the results of Comparative Example 2.

### Comparative Example 2

The procedure of Example 2 was repeated with the exception that trichloroethane was used as the solvent in the chromic acid chemical conversion treatment solution.

### Example 3

A phosphating treatment solution consisting of 100 parts methylene chloride, 36 parts methanol, 0.5 part orthophosphoric acid and 6 parts N,N-dimethyl formamide was kept at the boiling temperature thereof. Test panels of the same kind as used in Example 1 which had been degreased and cleansed beforehand were immersed in this boiling solution for 1 minute, thereafter they were dried in the vapor-free zone in the treating vessel. (Phosphating treatment)

Then, a chromic acid chemical conversion treatment solution consisting of 100 parts trichlorotrifluoroethane, 5 parts t-amyl alcohol and 0.5 part chromic acid anhydride was kept at the boiling temperature thereof, and the test panels which had been phosphated as described above were immersed in this boiling solution for 20 seconds, and then were dried in the vapor-free space. (Chromic acid chemical conversion treatment)

The thus treated panels were coated with a room-temperature-dryable acrylic resin paint ("Acrite No. 500" manufactured by Nippon Oil and Fats Co.) by air-spraying and dried at 80°C for 30 minutes. The primary adhesion and the corrosion resistance were tested and the results are indicated in Table 3.

### Comparative Example 3

The procedure of Example 3 was repeated with the exception that trichloroethylene was used as the solvent and 0.007 part zinc fluoride was added to the chromic acid chemical conversion treatment solution as a stabilizer. The results are indicated in Table 3 together with the results of Example 3. There was marked occurrence of blisters at the cross cutting, and the width of the peeled-off zone of the coating caused by the cellophane tape was broader.

### Example 4

The procedure of Example 3 was repeated with the exception that the panels were coated with a phthalic acid resin paint ("Glastone No. 1000" manufactured by Nippon Oil and Fats Co.) by spraying and were forcedly dried at 80°C for 30 minutes. The results are indicated in Table 4.

### Comparative Example 4

The procedure of Comparative Example 3 was repeated with the exception that the panels were coated with the phthalic acid resin paint used in Example 4 and was forcedly dried at 80°C for 30 minutes. The results are indicated in Table 4 together with the results of Example 4. The coating around the cross cutting was markedly damaged.

### Example 5

The procedure of Example 3 was repeated with the exception that the panels were coated with a melamine alkyd resin paint ("Melamine No. 1" manufactured by Nippon Oil and Fats Co.) by spraying and baked at 150°C for 20 minutes, and the panels were tested in the same manner as in Example 3. The results are indicated in Table 5.

### Comparative Example 5

The procedure of Example 3 was repeated with the exception that the panels were coated with the melamine alkyd resin paint used in Example 5 by spraying and baked at 150°C for 20 minutes and the panels were tested in the same manner. The results are indicated in Table 5.

### Example 6

A phosphating solution consisting of 100 parts trichlorotrifluoroethane, 22 parts methanol, 0.6 part orthophosphoric acid and 4 parts N,N-dimethylformamide was kept at the boiling temperature thereof. Test panels (70 x 150 x 0.8 mm galvanized steel sheets) which had been degreased and cleansed beforehand were immersed in the boiling solution for 1 minute, were thereafter washed with the vapor in the vapor zone above the treating solution and then dried in the vapor-free space. (Phosphating treatment).

Then, a chromic acid chemical conversion treatment solution consisting of 100 parts trichlorotrifluoroethane, 5 parts t-amyl alcohol and 1 part chromic acid anhydride was kept at the boiling temperature thereof. The test panels which had been phosphated as described above were immersed in this boiling solution for 15 seconds and dried in the vapor-free space. (Chromic acid chemical conversion treatment)

The thus treated panels were coated with an acrylic resin cationic electrodeposition paint ("Aqua No. 8000" manufactured by Nippon Oil and Fats Co.) by the conventional electrodeposition process, and baked at 170°C for 25 minutes.

The thus prepared painted panels were tested for the primary adhesion and then scored in the grid pattern and subjected to the corrosion test. The results are indicated in Table 6.

### Comparative Example 6

The procedure of Example 6 was repeated with the exception that methylene chloride was used as the solvent in the chromic acid chemical conversion treatment solution. The test results are indicated in Table 6 together with the results of Example 6.

## Claims

1. A process for treating metal surface comprising subjecting a metal surface to phosphating treatment and subjecting the phosphated surface to chromic acid chemical conversion treatment, said process being characterized in that the phosphating treatment is carried out using a non-aqueous phosphating treatment solution in which a chlorinated or chlorofluorinated hydrocarbon is used as the solvent and the chromic acid chemical conversion treatment is carried out using a non-aqueous chromic acid chemical conversion treatment solution in which a chlorofluorinated hydrocarbon is used as the solvent.

2. The process for treating metal surface as set forth in Claim 1, wherein the non-aqueous phosphating treatment solution comprises 100 parts by weight of a chlorinated or chlorofluorinated hydrocarbon, 0.05-5 parts by weight of a phosphoric acid compound, 1-75 parts by weight of an alcohol solubilizer having 1-20 carbon atoms, 0-2 parts by weight of nitrogen-containing organic compound reaction promoter and 0-15 parts by weight of aprotic polar compound; and the non-aqueous chromic acid chemical conversion treatment solution comprises 100 parts by weight of a chlorofluorinated hydrocarbon, 0.01-10 parts by weight of chromic acid anhydride, 0-0.1 parts by weight of an organic acid having 1-20 carbon atoms and 1-20 parts by weight of an alcohol solubilizer having 3-20 carbon atoms.

3. The process for treating metal surface as set forth in Claim 1, wherein in the phosphating treatment solution, the chlorinated or chlorofluorinated hydrocarbon is selected from a group consisting of carbon tetrachloride, chloroform, methylene chloride, 1,1,1-trichloroethane, trichloroethylene, perchloroethylene, trichlorotrifluoroethane, tetrachlorodifluoroethane, dichlorotetrafluoroethane, trichloromonofluoromethane, and mixtures of one or more thereof; the phosphoric acid compound is selected from a group consisting of orthophosphoric acid, pyrophosphoric acid, polyphosphoric acid, salts thereof, an acidic metal salt of phosphoric acid, an acidic alkyl ester of phosphoric acid, and mixtures thereof; the alcohol solubilizer is selected from a group consisting of methanol, ethanol, isopropyl alcohol, n-propanol, n-butanol, isobutanol and t-butanol; the nitrogen-containing organic compound is selected from a group consisting of urea, pyridine, thiourea, dimethyl isobutyleneamine, ethylenediamine tetraacetate and dinitrotoluene and the aprotic polar compound is selected from a group consisting of N,N-dimethylformamide, dimethylsulfoxide, acetonitrile, acetone, nitromethane, nitrobenzene and tetramethylenesulfone; and in the chromic acid chemical conversion treatment solution, the chlorofluorinated compound is selected from a group consisting of trichlorotrifluoroethane, tetrachlorodifluoroethane, dichlorotetrafluoroethane and trichloromonofluoromethane; the organic acid is selected from a group consisting of formic acid, acetic acid, lactic acid, stearic acid, oxalic acid, fumaric acid, maleic acid and malic acid; and the alcohol solubilizer is selected from a group consisting of isopropyl alcohol, n-propanol, tert-butanol, tert-amyl alcohol, triphenyl carbinol and mixtures of one or more thereof.

4. The process for treating metal surface as set forth in Claim 2 or 3, wherein the phosphating treatment solution contains a small amount of a stabilizer for the chlorinated hydrocarbon solvent selected from a group consisting of a quinone, an aromatic compound having a nitroso or azo functional group and a zinc compound.

5. The process for treating metal surface as set forth in Claim 4, wherein in the phosphating treatment solution, the chlorofluorinated compound is selected from methylene chloride and trichlorotrifluoroethane; the acid compound is selected from a group consisting of orthophosphoric acid, pyrophosphoric acid and polyphosphoric acid; the alcohol solubilizer is selected from a group consisting of methanol, ethanol, isopropyl alcohol and t-butanol; the nitrogen-containing organic compound is selected from a group consisting of dinitrotoluene, thiourea and dimethylisobutylenamine; and in the chromic acid chemical conversion the chlorofluorinated hydrocarbon solvent is selected from a group consisting of trichlorotrifluoroethane, tetrachlorodifluoroethane and trichloromonofluoromethane; the organic acid is selected from a group consisting of formic acid, fumaric acid, oxalic acid, acetic acid and lactic acid; the alcohol solubilizer is selected from a group consisting of t-butanol, t-amyl alcohol and isopropyl alcohol.

6. The process for treating metal surface as set forth in Claim 5, wherein the phosphating treatment solution consists of 100 parts by weight of methylene chloride or trichlorotrifluoroethane; 0.1-3.0 parts by weight of orthophosphoric acid or pyrophosphoric acid; 10-40 parts by weight of methanol, ethanol or t-butanol; 0.1-1 parts by weight of dinitrotoluene or thiourea; and 1-10 parts by weight of N,N-dimethylformamide or dimethylsulfoxide; and the chromic acid chemical conversion treatment solutions contains 100 parts by weight of trichlorofluoroethane or tetrachlorodifluoroethane; 0.07-2 parts by weight of chromic acid anhydride, 0.01-0.05 part by weight of formic acid, fumaric acid or oxalic acid.

## Revendications

1. Procédé de traitement d'une surface métallique comprenant le fait de soumettre une surface métallique à un traitement de phosphatation et le fait de soumettre la surface phosphatée à un traitement de conversion chimique par l'acide chromique, ledit procédé étant caractérisé en ce que le traitement de phosphatation est mis en oeuvre à l'aide d'une solution non aqueuse de traitement de phosphatation dans laquelle un hydrocarbure chloré ou chlorofluoré est utilisé comme solvant et le traitement de conversion chimique par l'acide chromique est mis en oeuvre à l'aide d'une solution non aqueuse de traitement de conversion chimique par l'acide chromique dans laquelle un hydrocarbure chlorofluoré est utilisé comme solvant.

2. Procédé de traitement d'une surface métallique selon la revendication 1, dans lequel la solution non aqueuse de traitement de phosphatation comprend 100 parties en poids d'un hydrocarbure chloré ou chlorofluoré, 0,05 à 5 parties en poids d'un composé de l'acide phosphorique, 1 à 75 parties en poids d'un agent de solubilisation alcoolique ayant 1 à 20 atomes de carbone, 0 à 2 parties en poids d'un promoteur de réaction qui est un composé organique contenant de l'azote et 0 à 15 parties en poids de composé polaire aprotique; et la solution non aqueuse de traitement de conversion chimique par l'acide chromique comprend 100 parties en poids d'un hydrocarbure chlorofluoré, 0,01 à 10 parties en poids d'anhydride chromique, 0 à 0,1 partie en poids d'un acide organique ayant 1 à 20 atomes de carbone et 1 à 20 parties en poids d'un agent de solubilisation alcoolique ayant 3 à 20 atomes de carbone.

3. Procédé de traitement d'une surface métallique selon la revendication 1, dans lequel, dans la solution de traitement de phosphatation, l'hydrocarbure chloré ou chlorofluoré est choisi dans un groupe formé par le tétrachlorure de carbone, le chloroforme, le chlorure de méthylène, le trichloro-1,1,1-éthane, le trichloréthylène, le perchloréthylène, le trichlorotrifluoroéthane, le tétrachlorodifluoroéthane, le dichlorotétrafluoroéthane, le trichloromonofluorométhane et les mélanges d'un ou de plusieurs de ceux-ci, le composé de l'acide phosphorique est choisi dans un groupe formé par l'acide orthophosphorique, l'acide pyrophosphorique, l'acide polyphosphorique, les sels de ceux-ci, un sel métallique acide de l'acide phosphorique, un alkylester acide de l'acide phosphorique et leurs mélanges, l'agent de solubilisation alcoolique est choisi dans un groupe formé par le méthanol, l'éthanol, l'alcool isopropylique, le n-propanol, le n-butanol, l'isobutanol et le t-butanol, le composé organique contenant de l'azote est choisi dans un groupe formé par l'urée, la pyridine, la thiourée, la diméthylisobutylenamine, le tétraacétate d'éthylènediamine et le dinitrotoluène et le composé polaire aprotique est choisi dans un groupe formé par le N, N-diméthylformamide, le diméthylsulfoxyde, l'acétonitrile, l'acétone, le nitrométhane, le nitrobenzène et la tétraméthylènesulfone, et dans la solution de traitement de conversion chimique par l'acide chromique, le composé chlorofluoré est choisi dans un groupe formé par le trichlorotrifluoroéthane, le tétrachlorodifluoroéthane, le dichlorotétrafluoroéthane et le trichloromonofluorométhane, l'acide organique est choisi dans un groupe formé par l'acide formique, l'acide acétique, l'acide lactique, l'acide stéarique, l'acide oxalique, l'acide fumarique, l'acide maléique et l'acide malique, et l'agent de solubilisation alcoolique est choisi dans un groupe formé par l'alcool isopropylique, le n-propanol, le tert-butanol, l'alcool tert-amylique, le triphénylcarbinol et les mélanges d'un ou plusieurs de ceux-ci.

4. Procédé de traitement d'une surface métallique selon la revendication 2 ou 3, dans lequel la solution de traitement de phosphatation contient une petite quantité d'un stabilisant pour le solvant hydrocarboné chloré choisi dans un groupe formé par une quinone, un composé aromatique ayant un groupe fonctionnel nitroso ou azo et un composé du zinc.

5. Procédé de traitement d'une surface métallique selon la revendication 4, dans lequel, dans la solution de traitement de phosphatation, le composé chlorofluoré est choisi parmi le chlorure de méthylène et le trichlorotrifluoroéthane, le composé acide est choisi dans un groupe formé par l'acide orthophosphorique, l'acide pyrophosphorique et l'acide polyphosphorique, l'agent de Solubilisation alcoolique est choisi dans un groupe formé par le méthanol, l'éthanol, l'alcool isopropylique et le t-butanol, le composé organique contenant de l'azote est choisi dans un groupe formé par le dinitrotoluène, la thiourée et la diméthylisobutylenamine, et, dans la conversion chimique par l'acide chromique, le solvant hydrocarboné chlorofluoré est choisi dans un groupe formé par le trichlorotrifluoroéthane, le tétrachlorodifluoroéthane et le trichloromonofluorométhane, l'acide organique est choisi dans un groupe formé par l'acide formique, l'acide fumarique, l'acide oxalique, l'acide acétique et l'acide lactique, l'agent de solubilisation alcoolique est choisi dans un groupe formé par le t-butanol, l'alcool t-amylique et l'alcool isopropylique.

6. Procédé de traitement d'une surface métallique selon la revendication 5, dans lequel la solution de traitement de phosphatation consiste en 100 parties en poids de chlorure de méthylène ou de trichlorotrifluoroéthane, 0,1 à 3,0 parties en poids d'acide orthophosphorique ou d'acide pyrophosphorique, 10 à 40 parties en poids de méthanol, d'éthanol ou de t-butanol, 0,1 à 1 partie en poids de dinitrotoluène ou de thiourée, et 1 à 10 parties en poids de N,N-diméthylformamide ou de diméthylsulfoxyde, et la solution de traitement de conversion chimique par l'acide chromique contient 100 parties en poids de trichlorofluoroéthane ou de tétrachlorodifluoroéthane, 0,07 à 2 parties en poids d'anhydride chromique, 0,01 à 0,05 partie en poids d'acide formique, d'acide fumarique ou d'acide oxalique.

## Patentansprüche

1. Verfahren zur Behandlung einer Metalloberfläche gemäß dem eine Metalloberfläche einer Phosphatierung unterworfen wird und die phosohatierte Oberfläche einer chemischen Umformungsbehandlung mit Chromsäure unterworfen wird, wobei das Verfahren dadurch gekennzeichnet ist, daß die Phosphatierung unter Verwendung einer nicht wässrigen Phosphatierungslösung in der ein chlorierter oder chlorfluorierter Kohlenwasserstoff als Lösungsmittel verwendet wird, durchgeführt wird, und die chemische Umformungsbehandlung mit Chromsäure unter Verwendung einer nicht wässrigen Chromsäurelösung zur chemischen Umformungsbehandlung in der ein chlorfluorierter Kohlenwasserstoff als Lösungsmittel verwendet wird, durchgeführt wird.

2. Verfahren zur Behandlung einer Metalloberfläche nach Anspruch 1, gemäß dem die nicht wässrige Phosphatierungslösung 100 Gewichtsteile eines chlorierten oder chlorfluorierten Kohlenwasserstoffs, 0,05 bis 5 Gewichtsteile einer Phosphorsäureverbindung, 1 bis 75 Gewichtsteile eines alkoholischen Lösungsvermittlers mit 1 bis 20 Kohlenstoffatomen, 0 bis 2 Gewichtsteile einer stickstoffhaltigen organischen Verbindung als Reaktionsbeschleuniger und 0 bis 15 Gewichtsteile einer aprotischen polaren Verbindung enthält; und die nicht wässrige Chromsäurelösung für die chemische Umformungsbehandlung 100 Gewichtsteile eines chlorfluorierten Kohlenwasserstoffs, 0,01 bis 10 Gewichtsteile Chromsäureanhydrid, 0 bis 0,1 Gewichtsteile einer organischen Säure mit 1 bis 20 Kohlenstoffatomen und 1 bis 20 Gewichtsteile eines alkoholischen Lösungsvermittlers mit 3 bis 20 Kohlenstoffatomen enthält.

3. Verfahren zur Behandlung einer Metalloberfläche nach Anspruch 1, gemäß dem für die Phosphatierungslösung der chlorierte oder chlorfluorierte Kohlenwasserstoff ausgewählt wird unter Tetrachlorkohlenstoff, Chloroform, Methylenchlorid, 1,1,1-Trichlorethan, Trichlorethylen, Perchlorethylen, Trichlortrifluorethan, Tetrachlordifluorethan, Dichlortetrafluorethan, Trichlormonofluormethan und Gemischen aus einer oder mehrerer dieser Verbindungen; die Phosphorsäureverbindung ausgewählt wird unter Orthophosphorsäure, Pyrophosphorsäure, Polyphosphorsäure, deren Salzen, einem sauren Metallsalz der Phosphorsäure, einem sauren Alkylester der Phosphorsäure, und deren Gemischen; der alkoholische Lösungsvermittler ausgewählt wird unter Methanol, Ethanol, Isopropylalkohol, n-Propanol, n-Butanol, Isobutanol und t-Butanol; die stickstoffhaltige organische Verbindung ausgewählt wird unter Harnstoff, Pyridin, Thioharnstoff, Dimethylisobutylenamin, Ethylendiamintetraacetat und Dinitrotoluol; und die arrotische polare Verbindung ausgewählt wird unter N,N-Dimethylformamid, Dimethylsulfoxid, Acetonitril, Aceton, Nitromethan, Nitrobenzol und Tetramethylensulfon; und gemäß dem für die Chromsäurelösung für die chemische Umformungsbehandlung die chlorfluorierte Verbindung ausgewählt wird unter Trichlortrifluorethan, Tetrachlordifluorethan, Dichlortetrafluorethan und Trichlormonofluormethan; die organische Säure ausgewählt wird unter Ameisensäure, Essigsäure, Milchsäure, Stearinsäure, Oxalsäure, Fumarsäure, Maleinsäure und Apfelsäure; und der alkoholische Lösungsvermittler ausgewählt wird unter Isopropylalkohol, n-Propanol, tert-Butanol, tert-Amylalkohol, Triphenylmethanol und Gemischen aus einer oder mehrerer dieser Verbindungen.

4. Verfahren zur Behandlung einer Metalloberfläche nach Anspruch 2 oder 3, gemäß dem die Phosphatierungslösung eine kleine Menge eines Stabilisators für das chlorierte Kohlenwasserstofflösungsmittel enthält, der ausgewählt wird unter einem Cuinon, einer aromatischen Verbindung mit einer funktionellen Nitroso- oder Azogruppe und einer Zinkverbindung.

5. Verfahren zur Behandlung einer Metalloberfläche nach Anspruch 4, gemäß dem für die Phosphatierungslösung die chlorfluorierte Verbindung ausgewählt wird unter Methylenchlorid und Trichlortrifluorethan; die Säureverbindung ausgewählt wird unter Orthophosphorsäure, Pyrophosphorsäure und Polyphosphorsäure; der alkoholische Lösungsvermittler ausgewählt wird unter Methanol, Ethanol, Isopropylalkohol und t-Butanol; die stickstoffhaltige organische Verbindung ausgewählt wird unter Dinitrotoluol, Thioharnstoff und Dimethylisobutylenamin; und gemäß dem für die Chromsäurelösung für die chemische Umformung das chlorfluorierte Kohlenwasserstofflösungsmittel ausgewählt wird unter Trichlortrifluorethan, Tetrachlordifluorethan und Trichlormonofluormethan; die organische Säure ausgewählt wird unter Ameisensäure, Fumarsäure, Oxalsäure, Essigsäure und Milchsäure; der alkoholische Lösungsvermittler ausgewählt wird unter t-Butanol, t-Amylalkohol und Isopropylalkohol.

6. Verfahren zur Behandlung einer Metalloberfläche nach Anspruch 5, gemäß dem die Phosphatierungslösung aus 100 Gewichtsteilen Methylenchlorid oder Trichlortrifluorethan, 0,1 bis 3,0 Gewichtteilen Orthophosphorsäure oder Pyrophosphorsäure, 10 bis 40 Gewichtsteilen Methanol, Ethanol oder t-Butanol, 0,1 bis 1 Gewichtsteilen Dinitrotoluol oder Thioharnstoff, und 1 bis 10 Gewichtsteilen N,N-Dimethylformamid oder Dimethylsulfoxid besteht; und die Chromsäurelösung für die chemische Umformungsbehandlung 100 Gewichtsteile Trichlorfluorethan oder Tetrachlordifluorethan, 0,07 bis 2 Gewichtsteile Chromsäureanhydrid, 0,01 bis 0,05 Gewichtsteile Ameisensäure, Fumarsäure oder Oxalsäure enthält.
